

Patented Apr. 10, 1928.

1,665,500

# UNITED STATES PATENT OFFICE.

ISADORE M. JACOBSON, OF CHICAGO, ILLINOIS, AND STARR TRUSCOTT, OF BIRMINGHAM, OHIO.

## AIRCRAFT COVERING.

No Drawing.

Application filed April 11, 1925. Serial No. 22,347.

This invention relates to improvements in flexible gas retaining fabrics for aircraft and more particularly to the gas retaining fabric used in the gas cells of aircraft of the Zeppelin type.

One of the objects of the present invention is to provide an impermeable flexible membrane or fabric of the above general character which may be inexpensively manufactured and fabricated into gas retaining bags or cells.

A further object is to provide a fabric of the above general character adapted to eliminate the use of goldbeaters skins heretofore considered essential.

Other objects will be in part obvious and in parts hereinafter pointed out.

The disadvantages of a gas retaining fabric using goldbeaters skin as an impermeable film has been described in our pending specification filed Apr. 11, 1925, Serial No. 22346 for a fabric using cellulose or sheet viscose as a substitute for the goldbeaters skin. The fabric described hereafter is intended to overcome the disadvantages incident to the preparation of goldbeaters skin fabric in another manner.

It has been found that a film produced from a mixture of viscose and latex has a very high resistance to the passage of gases. Such material can be produced either in large sheets or spread directly on cloth in a manner similar to that in which rubber is applied. We have prepared and tested many samples of fabric using this film prepared from the mixture of latex and viscose and found them to be satisfactory for this purpose.

A fabric treated with our invention is not only impermeable to gases but also is extremely flexible, being equally as pliable as goldbeater's skin and therefore is particularly adapted for the purpose designed.

The following example will illustrate the method of preparing gas impermeable fabrics from a mixture of viscose and latex. Dissolve 0.29 gms. of tetramethyl thiuram disulfide in 15 cc. of acetone. Add this solution quickly to 400 cc. of water at 20° C. This is immediately followed by the addition, with vigorous agitation, of 70 gms. of rubber latex containing 40% of solid matter. It is essential that this operation be very quickly carried out in order to prevent the coagulation of the first substance added.

Three gms. of zinc sulphate, dissolved in 10 cc. of water, are treated with 7 cc. of ammonia water containing 29% of ammonia. The white precipitate which is formed at first should be completely redissolved before proceeding further. This solution is then added to the latex solution above, agitating well. Two hundred and fifty gms. of viscose are then added to this mixture and stirred well until a homogeneous solution results. The viscose used must not have aged excessively at the time of use. Swollen fibrous particles will separate from a mixture of old viscose and latex. The length of time such viscose solutions may be kept without excessive deterioration depends upon the temperature at which they are kept, decomposition occurring more rapidly at higher temperatures. We have found it possible, however, to use viscose which had been stored in a glass vessel kept in an ice chest for as long as 15-20 days. The viscose-latex mixture prepared by the above method should be kept at a temperature not exceeding 20° C. until applied.

In order to prepare a gas impermeable flexible fabric from the viscose-latex mixture, the fabric is first sized with a suitable gelatine or glue adhesive for the viscose-latex film that is later built upon it. The viscose-latex mixture, prepared as outlined above, is then spread upon the sized fabric, a total of eight to fifteen coats being spread, depending upon the impermeability and weight desired. Each coat is dried by passing a current of air at a temperature of 40° C. over its surface before the application of the next coat. When the last coat is dry, the fabric is passed through a bath composed of an aqueous solution containing 25% magnesium sulphate at a temperature of 30°-40° C. The duration of this procedure depends upon the exact temperature used, the fabric being left in this bath until it acquires a uniform tan color. It is then passed through a bath containing a 2% aqueous solution of sodium bisulphite until it becomes white in color. After this it is washed with cold water to remove water soluble salts and passed through a bath containing 15% of glycerine by volume. The fabric is then allowed to drain and dry. The fabric thus obtained is light in weight and virtually impermeable to gases. After standing for several weeks, it acquires greater

strength and becomes sufficiently flexible to withstand wrinkling without any noticeable increase in permeability.

It must be understood that we do not limit ourselves to the use of proportions of the various ingredients specified in the above example. Furthermore, we do not limit ourselves to the use of the accelerator, tetramethyl thiuram disulphide, or the use of the activator, zinc sulphate, or the temperatures specified in this example. We reserve also the right to change the order in which the various ingredients may be added in preparing the viscose-latex mixture.

15 It will thus be seen that the present invention provides a simple and practical flexible gas retaining fabric for use on aircraft adapted to accomplish, among others, all of the objects and advantages herein set forth.

20 What we claim is:—  
1. A method of rendering a fabric impermeable to gases and flexible consisting in applying an adhesive agent to said fabric, superimposing thereon a plurality of layers 25 of viscose-rubber latex solution, and passing said coated fabric first through a bath of magnesium sulphate then through a bath of sodium bisulphite, then of clear water, and finally of glycerine, to convert the film of 30 viscose-latex into one of cellulose-rubber and to render the coating insoluble in water and to render it flexible.

2. A method of rendering a fabric imper-

meable to gases and flexible consisting in applying an adhesive to said fabric, applying thereupon a plurality of layers of viscose-rubber latex solution drying each layer before applying the next, and passing the finally dried coated fabric first through a bath of magnesium sulphate then through a 40 bath of sodium bisulphite, then of clear water, and finally of glycerine, to convert the film of viscose-latex into one of cellulose-rubber and to render the coating insoluble in water and to render it flexible. 45

3. A method of treating a fabric to render the same flexible and impermeable to gases consisting in applying an adhesive to the fabric, superimposing thereupon a plurality of layers of viscose-rubber latex solution, 50 drying each layer before applying the next, bathing the finally dried coated fabric in a solution of magnesium sulphate, bathing in a solution of sodium bisulphite, removing soluble salts therefrom, passing it through 55 a bath containing glycerine, draining and drying.

4. A fabric coated with gelatine having a viscose-rubber latex superimposed thereupon and treated with a plasticizing agent, whereby the fabric is rendered flexible and impermeable to gases. 60

Signed at Washington, District of Columbia, this 9th day of January, 1925.

ISADORE M. JACOBSON.  
STARR TRUSCOTT.